

March 16, 1948.

C. FRONDEL

2,437,913

QUARTZ OSCILLATOR PLATE

Filed Dec. 15, 1944

*Fig. 1*



*Fig. 2.*



INVENTOR  
CLIFFORD FRONDEL

*Penile, Davis, Marvin Edmonds*  
BY  
ATTORNEYS

## UNITED STATES PATENT OFFICE

2,437,913

## QUARTZ OSCILLATOR PLATE

Clifford Frondel, Flushing, N. Y., assignor to  
 Reeves-Ely Laboratories, Inc., New York, N. Y.,  
 a corporation of New York

Application December 15, 1944, Serial No. 568,326

17 Claims. (Cl. 171—327)

1

This invention relates to quartz oscillator plates and has for its object certain improvements in the method of manufacturing oscillator plates made of quartz or equivalent material.

In the manufacture of so-called BT quartz oscillator plates, for example, automatic or semi-automatic machines are generally employed in the initial and intermediate states. The final finishing of the plates is, however, still largely a hand operation, the work being done by highly skilled operatives, usually called finishers. In finishing the plates, physical dimensions of the order of sub-millionths of an inch are involved. The finisher is usually provided with a frequency-checking device, a flat glass plate, fine abrasive, an etching solution, water, a brush, cleaning solutions, lint-free towels, a micrometer, an optical flat, a small square, etc.

The finisher receives the plates, sometimes called blanks, as they come from mechanical lapping machines, the plates having been cut to substantially proper length and width and usually brought close to, but less than, the desired oscillating frequency. In a plate desired to have a final frequency of, say, 8,000 kc., the machine lapping or other pre-hand-finishing treatment is stopped when the plate is from roughly a few hundred cycles up to ten or more kilocycles under the final desired frequency. A preliminary frequency check is then made by comparing the frequency of the plate with that of a standard plate having a known frequency. This gives the finisher a general idea how much hand lapping the plate should be given. To reduce the plate to its proper thickness, and hence to increase its frequency, the finisher grinds the plate in a mixture of the abrasive and water on the flat glass plate, keeping the faces of the plate as flat and parallel as possible. The plate is next thoroughly cleaned and dried, after which its frequency is again tested. This is done by inserting the carefully cleaned plate in a holder, plugging the holder into an oscillator circuit and noting whether or not the plate has reached the desired oscillating frequency. The lapping of the major plane surfaces of the plates usually is accompanied by a lapping or beveling of the edges of the plates; this operation, by removing roughness and other imperfections from the edges and by altering the edge dimensions, gives the desired degree of activity, so-called, to the plate.

The finishing of a plate to its desired frequency also may be accomplished in other ways, and a number of techniques other than hand lapping have been and are being developed in the oscil-

2

lator-plate industry. Thus, in the so-called acid-dip or etching process, the plates as obtained at the completion of the machine lapping are brought up to the desired frequency by dipping them for the required length of time into a solvent for quartz. This solvent, which may be, for example, hydrofluoric acid, removes quartz from the surface of the plate and thus acts to reduce the thickness of the plate to the desired value. This process, as with hand lapping, requires an intermittent, successive, series of treatments and measurements, especially in the final stages, to ensure that the desired frequency is exactly attained. The rate of etching of different plates of the same initial frequency is not identical, due to variations in the cleanliness of the surface, the roughness of the surface, and other factors, so that a uniform, timed, procedure for all plates cannot be set out. In still another method of finishing plates to the desired frequency, the plates are tumbled with an amount of coarse abrasive in a container until the frequency approaches that desired. The plates are then removed, cleaned, and are adjusted to the desired frequency either by etching or hand lapping.

Alternate hand lapping, cleaning and testing are required until the plate reaches the desired frequency. The activity of the plate is determined by its dimensions, contour, parallelism, absence of flaws, cleanliness, etc. These physical characteristics are checked, changed, and rechecked until the desired activity is obtained. The frequency of the plate changes with changes made in the plate to obtain the desired activity, so that the finisher must coordinate the numerous variables going into the finishing operation to obtain a combination of conditions that yields a plate of predetermined activity and frequency.

Hand finishing by these methods of the oscillator plates is a tedious, slow, delicate and costly operation at best and leaves much to be desired. The human factor is an exceedingly important element in these finishing operations and the results obtained tend naturally to vary from person to person, depending upon the particular technique employed at the time by each finisher.

As a result of my investigation I have discovered that the frequency and certain other characteristics of piezo-electric bodies may be adjusted or varied without altering the physical dimensions of the body, such as by grinding, etching or plating with a metal or other material. The frequency of oscillation of quartz oscillator plates, for example, may be varied continuously and this variation may be brought under continu-

ous visual control as by an appropriate meter. This permits the frequency to be adjusted exactly to a predetermined value or range merely by following the frequency variation on a meter and stopping the treatment at the desired value or within the desired range. This is not possible in present methods of manufacture of piezo-electric bodies which, as noted above, involve a discontinuous alternating process of grinding or etching, cleaning and testing. The frequency of oscillation of quartz oscillator plates may, for example, be readily adjusted to a desired value with an accuracy up to 1 cycle or greater, depending primarily on the accuracy of the measuring device employed. This accuracy cannot be accomplished by the conventional method of grinding or etching because the amount of grinding or etching on which the change of frequency and accuracy depends cannot be accurately controlled or measured, and the change in frequency itself cannot be observed continuously.

The frequency of a piezo-electric body that has been put into a relatively stable state by means of baking, etching with a solvent for quartz, or other treatment, such as for the purpose of eliminating or reducing spontaneous variation with time in the frequency or activity of the piezo-electric body, can be adjusted without destroying the stability of the piezo-electric body. This is not possible by present methods of manufacture. For example, if a number of quartz oscillator plates are brought by grinding or etching to a desired frequency, and are then baked or otherwise treated, for the purpose of stabilization, it is found that the frequency often changes erratically from the original value and must then be adjusted by additional grinding or etching. This action then destroys the stability of the oscillator plate and the purpose of the original stabilizing operation is lost. This readjustment can now be accomplished without grinding or etching and without loss of stability.

The frequency of oscillator plates may be adjusted, for example, without wetting them with water or other liquids and in an entirely dry condition. Water is commonly used in the conventional method of finishing to frequency by lapping with an abrasive or by etching, and has been considered to contribute substantially to undesirable ageing and other phenomena in the finished oscillator plate. This difficulty may now be obviated.

The frequency of a piezo-electric body can be adjusted while it is contained in its permanent holder, whether this is of the contact (pressure), air gap, wire suspension or other type of mount. If desired, the frequency of the piezo-electric body may be adjusted before it is mounted in its permanent holder.

The change in frequency brought about by application of the invention is downwards from the initial value, but the downwards change may be reversed, and the frequency restored to its original value, by suitable treatment. The new technique is especially advantageous in the recovery of oscillator plates that have been overshot by the ordinary methods of hand finishing. Oscillator plates that have increased in frequency over the upper tolerance due to ageing, or aged low activity plates that have gone over the tolerance after cleaning to bring up the activity, may be similarly readjusted to their original frequency.

In accordance with the invention, the method comprises the step of treating quartz oscillator plates to the action of radio-active emanations

adapted to decrease their frequency of oscillation.

The radio-active emanations may be derived from such radio-active substances as radium, radon, uranium, polonium, actinium and thorium. Three different types of radiation are released spontaneously during radio-active disintegration. They are (1) positively charged particles, called alpha particles; (2) negatively charged particles, called beta particles; and (3) uncharged non-corporeal rays, called gamma rays. Alpha particles cause intense ionization as they traverse a gas; they have a relatively slow speed, are weakly penetrating and are readily absorbed by solids. Beta particles are relatively high speed electrons which ionize a gas, although not so intensely as alpha particles, and are much more penetrating than alpha particles. Gamma rays are electromagnetic rays of the same nature as X-rays but for the most part of much shorter wave length. They are very much more penetrating than the alpha and beta particles. They ionize a gas through which they pass, the ionization being largely due to an emission of secondary beta particles which result whenever gamma rays traverse matter.

The radium salts and the radio-active gas preparations ordinarily used in medical work, when in radio-active equilibrium, afford all three types of radiation, but the glass or metal capsules used to hold the radium salt or gas preparations effectively screen off the alpha particles. Alpha radiation is conveniently applied by sealing the quartz oscillator plates in a container filled with radon gas, an intermediate member of the radium disintegration series, or directly in a container partially filled with a radium salt. Containers having glass or metal walls of appropriate thickness may be used to hold back both alpha and beta particles and to permit emission of the gamma rays; so that the oscillator plates may be directly exposed to the gamma rays.

As pointed out in my co-pending application Serial No. 568,323, filed December 15, 1944, the change in frequency produced in oscillator plates by the radio-active emanations is downwards from the original value. The change is progressive and continuous during irradiation but finally reaches a limiting value, determined by factors within the quartz, beyond which there is no further change. The rate of change appears to depend primarily on the intensity of the radiation, but in part on variations in the properties of the quartz from specimen to specimen and on pre-treatment of the quartz. The continuity of the change is of great importance from a manufacturing point of view. The downward direction of the change is also of particular advantage.

The downward change in frequency brought about by the radio-active emanations is permanent under ordinary conditions, but can be reversed and the oscillator plate brought back to its original frequency by baking at a suitably elevated temperature or by irradiating the plate with ultra-violet rays. Ultra-violet rays reverse the action of the other type of radiation. The ability to reverse the downward change is a great advantage. In other words, the oscillator plates may be adjusted downwards and upwards in frequency repeatedly by the proper treatment.

The rate at which the downward change in frequency of the oscillator plates can be effected and the total amount of change is influenced by the temperature at which the quartz is held

during irradiation, and by previously baking the quartz at a suitably elevated temperature.

These and other features of the invention will be better understood by referring to the accompanying drawing, taken in conjunction with the following description, in which:

Fig. 1 is a vertical cross-sectional view of a container showing a plurality of quartz oscillator plates stacked therein for treatment with radioactive emanations; and

Fig. 2 is a vertical cross-sectional view of a similar container showing a plurality of spaced quartz oscillator plates suspended therein and connected to a frequency meter.

Referring first to Fig. 1, the apparatus shown comprises a container 10 having a chamber 11 defined by thick walls 12, preferably of lead not less than  $1\frac{1}{4}$  inches thick. A suitable removable metal rack 13 provided with legs 14 fits within chamber 11, a plurality of quartz oscillator plates 15, 15', 15'', etc., being stacked therein. A plunger 16 extends through the side wall of the container into and near the bottom of chamber 11. The bottom of the chamber is provided with a fixed stop 17 against which a capsule 18 of radioactive material may be disposed in alignment with the plunger. The top of the container is fitted with a cap 19 of the same thick-walled material, the cap preferably fitting tightly over the container to prevent the escape of radio-active material or emanations therefrom.

Referring next to Fig. 2, the apparatus shown comprises a similar container 10, except that its chamber 11 is preferably wide enough to accommodate a plurality of spaced quartz oscillator plates 15, 15', 15'', suspended from cap 19 in the manner indicated. Each oscillator plate is mounted in what amounts to a holder, or part of a holder, of the wire-support type. The ends of a pair of wires 20 and 21 are suitably secured to the major faces of each oscillator plate, the wires in turn being secured to a support or base 22 as well as being in electrical contact with a corresponding pair of terminals 23 and 24, respectively.

Terminals 23 and 24 of the holder are insertable in and removable from sleeves 25 and 26, respectively, within cap 19. These sleeves are, in turn, connected to a frequency meter 27 by means of leads 28 and 29. The frequency meter may be of conventional design having a needle 30 adapted to move back and forth over a graduated frequency scale 31, preferably divided to indicate cycles per second.

In operating the apparatus of Fig. 1, a capsule 18 of radio-active material is disposed between stop 17 and the end of plunger 16. A stack of quartz oscillator plates 15, 15', 15'', is fitted within rack 13, which is then placed in position within chamber 11. Cap 19 is placed over the container and plunger 16 is pushed inwardly with sufficient force to break capsule 18, thus permitting radio-active emanations to escape therefrom. As the radio-active emanations diffuse throughout the container, they act upon the oscillator plates. This container is used if it is not desired to oscillate the quartz oscillator plates during the time of their irradiation.

In operating the apparatus of Fig. 2, capsule 18 is similarly placed between stop 17 and the end of plunger 16. Quartz oscillator plates 15, 15', 15'' are suitably suspended from wires 20 and 21, and terminals 22 and 23 are pushed into contact sleeves 25 and 26, respectively. Cap 19

is then placed on the container and plunger 16 is pushed inwardly to break capsule 18. The plates may be oscillated continuously or intermittently while exposed to the resulting radioactive emanations, so that the frequency change can be measured by means of frequency meter 27. When the plates acquire the desired oscillating frequency value or range, cap 19 is removed from the container.

10 In accordance with the invention, quartz oscillator plates were exposed for periods up to 37 days to radium salt preparations contained in thin tubes which screened off the alpha rays. Also, oscillator plates were exposed for periods up to 30 days in radon gas; in this case some of the plates were so mounted in the container as to permit them to be oscillated and their frequency measured during exposure to the radiations. The oscillator plates decreased in frequency in the case of gamma radiation, but smaller total changes were brought about by the beta and especially the alpha radiations due to their only partial penetration (range) into the quartz. The alpha and beta particles, however, because of their relatively great ionizing power, effect a frequency change much more rapidly than do the gamma rays. Thus, in spite of the smaller total change that they can effect, they may be more useful from a manufacturing point of view than the gamma radiation. It was found that irradiated plates gave X-ray Laue transmission patterns indistinguishable from those of non-irradiated plates.

Radon is one of the radio-active disintegration products proceeding from uranium and radium and ultimately ends in the Ra G isotope of lead. The members of the disintegration series, with the exception of the end-product, lead, are unstable and transform successively into the next member at definite rates. The transformation is accompanied by the emission of radiations, either alpha particles or beta particles plus gamma rays. Radon itself emits only alpha particles, but the freshly prepared gas progressively disintegrates into Ra A, Ra B, etc., all present simultaneously in a state of transient equilibrium, and some of these contribute beta and gamma radiations. Because of the long half-life period of Ra D, 25 years, and the extremely short life of the intermediate disintegration products between radon and Ra D, the length of time in which a radon preparation can be used as a practical source of radiation is fixed by the disintegration constant of radon itself.

In using radon to adjust frequency of oscillation, the plates are sealed in a hollow lead container in direct contact with the gas where they are acted upon by the alpha, beta and gamma radiations proceeding therefrom. The walls of the container should be at least one inch thick to guard against escape of the gamma rays. Ordinarily, the container is opened and the plates removed while a considerable portion of the original radon charge still remains. This operation should be done in a hood under strong ventilation. After irradiation the plates should be allowed to stand for 30 minutes or more before handling so that the activity of the solid radio-active decomposition products on their surface has time to diminish to a negligible value. Care also must be taken in loading the lead container with radon. The gas is supplied in capillary glass tubes a centimeter or so long sealed within larger glass tubes which in turn

are housed in a lead bottle. When removing the radon tube from the lead bottle for use, it should be handled with long tweezers. The lead irradiation container should be so arranged as to permit breaking the radon tube within it after sealing. If the capillary tube is not broken the glass walls cut off the alpha and most of the beta radiation.

The curves obtained by plotting the frequency change against time of exposure or millicurie-hour exposure differ from the X-ray curves in several respects. The radon curves fall into two parts: an initial period of rapid change which comprises only part of the total frequency change that can be effected, followed by a slow and relatively uniform change that apparently continues to saturation. The initial rapid change seems caused by strongly ionizing radiations of only limited penetration in quartz which rapidly saturate a certain thickness and thereafter are ineffective. These radiations appear to comprise the alpha and beta particles. The period of slow uniform change apparently represents ionization by the extremely penetrating but very weakly absorbed gamma radiation. It is also found that the magnitude of the initial bump in the curve increases with increasing concentration of the radon. This effect seemingly is due to an increase in the average penetrating power of the radiation. The increase may arise in the shorter average path distance of the radiation in the air of the container as the radon concentration increases, with consequent less loss of energy by absorption and scattering before entering the quartz.

Theoretically, the time rate of change of frequency should vary in proportion to the concentration of radon, and the millicurie-hour rate of change in plates of a given frequency should be constant and independent of concentration. There are rather marked departures from this due to intrinsic variations in the response of different specimens of quartz and to the penetration effect noted above. The average millicurie-hour rate of change of frequency calculated from the limited data at hand is roughly 2.26 cycles per mc.-hr. in 8163 kc. plates. The rate was calculated on the basis of the initial, linear, part of the frequency curves.

The advantage of the radon method is that a large number of plates can be equally and simultaneously irradiated. This can be accomplished by racking the plates in the container. The unit cost is proportional to the number of plates, since the same amount of radon will suffice for one as for many plates, within certain limits, if the gas volume is kept constant by appropriate design of the rack and container. This is due to the fact that only a small part of the available radiation is utilized in any case. The principal factors that determine the application of the method are the cost of the radon, the total number of plates to be irradiated, the average amount of frequency change desired, and the time in which the frequency change must be effected. The two latter factors fix the amount of radon that must be employed. The actual estimation of this amount requires a knowledge of the relation between radon concentration and both the average amount of frequency change and the average time rate of change of frequency. These two factors are not independent, as noted, and their relation to radon concentration varies with the frequency of the plate. The amount of radon required, the exposure time, and the accompanying total

average frequency change can be calculated directly if any one of these factors is known and if the millicurie-hour rate of change of frequency has been previously established for the plate frequency in question and the container in question. The use of radon is more particularly described and claimed in my co-pending application Serial No. 568,327, filed December 15, 1944.

The rate of change of frequency during irradiation is rapid, at first, but drops off with time and distance, finally to approach a limiting value. The magnitude of the limiting value varies with different specimens of quartz. This variation, which in the extreme cases so far encountered is about tenfold, appears to depend primarily on a predisposing feature in the quartz itself. The actual rate of change in frequency in a given oscillator plate varies with the conditions of treatment, and primarily with the intensity of radiation. The decrease in frequency during irradiation is accomplished with little, if any, significant change in activity.

An oscillator plate that has been baked at an elevated temperature is found when subsequently irradiated to change frequency more rapidly. The increase in rate brought about by baking between 250° and 350° C. ranges up to twofold, and there is an accompanying increase in the total frequency range. It is often advantageous to heat the plates to 300° to 570° C. in order markedly to sensitize them prior to irradiation with X-rays. Such baking has a stabilizing effect on the irradiated plates. In this connection it may be noted that a former objection to the baking of the plates, that of erratic increase in frequency which often brought the plates out of tolerance, is readily overcome by the irradiation method without destroying the stability of the plates.

As previously noted, the frequency of quartz oscillator plates also undergoes a change when the plates are treated with ultra-violet rays; the change in frequency, however, being upwardly instead of downwardly. Oscillator plates irradiated as described above in order to decrease their frequency may be reverted in frequency to their initial value when exposed, for example, to a powerful quartz-mercury lamp. The change is accelerated by heating the quartz oscillator plates to 100-150° C. during irradiation with the ultra-violet rays.

The use of ultra-violet rays offers an important advantage. If for some reason the frequency of an oscillator plate should be decreased too much by the other type of radiation disclosed, its frequency may be increased to the desired value. The use of ultra-violet light rays is more particularly described and claimed in my co-pending application Serial No. 568,330, filed December 15, 1944.

It will be clear to those skilled in this art that the invention lends itself to numerous modifications. The oscillator plates may be irradiated whether plated or unplated, coated or uncoated. In accordance with the invention the oscillator plates may, for example, be plated with a metal such as gold, silver, aluminum or an alloy which may serve the purpose of making a better or more intimate electrical contact with or act as electrodes; or which may serve as protective or stabilizing films. The plates may, for example, be coated with amorphous silica or organic plastic or other material which may serve the purpose of protective or stabilizing films. In the case of oscillator plates that have been protected or sta-

bilized by a plating, coating or other treatment, including heating and ageing, the radiations herein contemplated are adapted nevertheless to modify the oscillator plates so as to vary their oscillating characteristics; and irradiation of the plates may be conducted until their frequency of oscillation reaches the desired value without substantial loss of stability. The plates may be adjusted upwards or downwards in frequency repeatedly by use of the proper radiations.

It also is possible to adjust the plate to have a desired frequency at a given temperature by irradiating the plate, and bringing it to frequency, while it is held at that temperature in a suitable heating or cooling contrivance. This is not easily accomplished by the conventional lapping or etching techniques of finishing plates.

The rate of change of frequency of the plate during irradiation and also the total amount of frequency change that can be obtained (saturation value) can be modified by baking the quartz plate at a suitable temperature before it is irradiated. Thus, baking the quartz plate at a suitably elevated temperature has been found to increase both the rate of change and the amount of change of frequency over that which would obtain if the plate had not been baked beforehand.

The oscillator plates may be irradiated whether mounted or unmounted. It is advantageous to irradiate the plates while they are mounted in a temporary or permanent holder and while the plates are oscillating. It is particularly advantageous to conduct the irradiation operation while the oscillator plates are mounted in a permanent holder connected with a suitable meter, so that the change in frequency of oscillation which takes place may be visually observed and the irradiation stopped when the plates have attained the desired frequency. The type of permanent holder, for example, may be of the pressure or clamp, air-gap, combined pressure and air-gap, wire-support, mechanically or hermetically sealed, temperature-controlled or temperature protected, or the multiple-type. If the oscillator plates are mounted in a permanent holder, the radiations go right through the plastic, glass or metal shell, or housing of the holder. A sufficiently penetrating radiation must, of course, be employed. This practice is especially useful in the case of oscillator plates supported between wire suspension mounts in thin-walled vacuum holders. If the oscillator plates are not mounted in a holder, they may be held, for example, in paper or aluminum foil envelopes which protect them from moisture, dust and grease spots from handling.

It also is convenient under certain circumstances to irradiate a large number of plates simultaneously. This can be done, for example, by stacking the plates together and placing the stack directly in front of the window, face on. The amount of frequency change thus brought about is not uniform through the stack, but is greatest in the first plate, considerably less in the second, and then decreases more slowly in succeeding plates.

A further technique of irradiation that may be practiced to advantage consists of temporarily or permanently mounting a quartz oscillator plate within a Bakelite or other conventional holder and introducing an amount of radio-active material or gas therein. The radio-active material is allowed to act on the quartz plate until the frequency is adjusted to the desired range or value and is then removed or flushed from the holder and the action thereby stopped. Alternatively, a

definite amount of radio-active material may be permanently sealed within the holder, to afford during the radio-active life period of the material the amount of radiation calculated to be necessary to reduce the frequency of the quartz plate to a desired range or value. Further, an amount of radio-active material of extremely long life, such as radium element or a salt of radium, may be permanently sealed within the holder to compensate downwards any upwards drift in frequency that may result from excessive heating or otherwise.

While the practice of the invention has been described with respect to piezo-electric material in the form of quartz, it will also be clear to those skilled in this art that the invention is applicable to the treatment of other piezo-electric materials, such as Rochelle salts, tourmaline, tartrates, etc. The invention is applicable to the treatment of any useful piezo-electric material the frequency and oscillating characteristics of which are to be varied under controlled conditions.

I claim:

25. 1. In the manufacture of quartz oscillator plates, the improvement which comprises treating each oscillator plate with radiations from a radio-active substance adapted to decrease its frequency of oscillation.
30. 2. In the manufacture of quartz oscillator plates, the improvement which comprises treating each oscillator plate with radiations from a radio-active substance adapted to decrease its frequency of oscillation, and terminating the treatment of each plate with said radiations from the radio-active substance when its frequency of oscillation reaches a predetermined value.
35. 3. In the manufacture of quartz oscillator plates, the improvement which comprises treating each oscillator plate while mounted in a holder connected to a frequency meter to the action of radiations from a radio-active substance adapted to decrease the frequency of oscillation of the plate, and terminating the treatment of each plate with said radiations from the radio-active substance when its frequency of oscillation reaches a predetermined value.
40. 4. In the manufacture of quartz oscillator plates, the improvement which comprises treating each plate while mounted in a holder connected to a frequency meter to the action of radiations from a radio-active substance adapted to pass through the housing of the holder and to decrease the frequency of oscillation of the plate, and terminating the treatment of each plate with said radiations from the radio-active substance when its frequency of oscillation reaches a predetermined value.
45. 5. In the manufacture of quartz oscillator plates, the improvement which comprises maintaining each oscillator plate at a predetermined temperature, treating each plate while at said temperature with radiations from a radio-active substance adapted to decrease its frequency of oscillation, and terminating the treatment of the plate with said radiations from the radio-active substance when its frequency of oscillation reaches a predetermined value.
50. 6. In the manufacture of quartz oscillator plates, the improvement which comprises maintaining each oscillator plate at a predetermined temperature while mounted in a holder connected to a frequency meter, treating the plate while at said temperature with radiations from a radio-active substance adapted to decrease the frequency of oscillation reaches a predetermined value.
55. 7. In the manufacture of quartz oscillator plates, the improvement which comprises maintaining each oscillator plate at a predetermined temperature while mounted in a holder connected to a frequency meter, treating the plate while at said temperature with radiations from a radio-active substance adapted to decrease the frequency of oscillation reaches a predetermined value.
60. 8. In the manufacture of quartz oscillator plates, the improvement which comprises maintaining each oscillator plate at a predetermined temperature while mounted in a holder connected to a frequency meter, treating the plate while at said temperature with radiations from a radio-active substance adapted to decrease the frequency of oscillation reaches a predetermined value.
65. 9. In the manufacture of quartz oscillator plates, the improvement which comprises maintaining each oscillator plate at a predetermined temperature while mounted in a holder connected to a frequency meter, treating the plate while at said temperature with radiations from a radio-active substance adapted to decrease the frequency of oscillation reaches a predetermined value.
70. 10. In the manufacture of quartz oscillator plates, the improvement which comprises maintaining each oscillator plate at a predetermined temperature while mounted in a holder connected to a frequency meter, treating the plate while at said temperature with radiations from a radio-active substance adapted to decrease the frequency of oscillation reaches a predetermined value.

quency of oscillation of the plate, and terminating the treatment of each plate with said radiations from the radio-active substance when its frequency of oscillation reaches a predetermined value.

7. In the manufacture of quartz oscillator plates, the improvement which comprises maintaining each oscillator plate at a predetermined temperature while mounted in a holder connected to a frequency meter, treating each plate to the action of radiations from a radio-active substance adapted to pass through the housing of the holder and to decrease the frequency of oscillation of the plate, and terminating the treatment of each plate with said radiations from the radio-active substance when its frequency of oscillation reaches a predetermined value.

8. In the manufacture of quartz oscillator plates, the improvement which comprises grinding each oscillator plate to a thickness beyond that required to increase its frequency to a predetermined value, and treating each ground plate with radiations from a radio-active substance adapted to decrease its frequency of oscillation.

9. In the manufacture of quartz oscillator plates, the improvement which comprises grinding each oscillator plate to a thickness beyond that required to increase its frequency to a predetermined value, treating each ground plate with radiations from a radio-active substance adapted to decrease its frequency of oscillation, and terminating the treatment of each ground plate with said radiations from the radio-active substance when its frequency of oscillation reaches a predetermined value.

10. In the manufacture of quartz oscillator plates, the improvement which comprises etching each oscillator plate to a thickness beyond that required to increase its frequency to a predetermined value, treating each etched plate with radiations from a radio-active substance adapted to decrease its frequency of oscillation, and terminating the treatment of each etched plate with said radiations from the radio-active substance when its frequency of oscillation reaches a predetermined value.

11. In the manufacture of quartz oscillator plates that have been stabilized by baking, acid washing or other treatment and that have a frequency of oscillation higher than desired, the improvement which comprises treating each stabilized oscillator plate with radiations from a radio-active substance adapted to decrease its frequency of oscillation, and terminating the treatment of each stabilized plate with said radiations from the radio-active substance when its frequency of oscillation reaches a predetermined value.

12. In the manufacture of quartz oscillator plates, the improvement which comprises treating each oscillator plate with radiations from a radio-active substance adapted to decrease its frequency of oscillation, heating each oscillator plate so treated to increase its frequency of oscillation, and terminating the heating of each plate when its frequency of oscillation reaches a predetermined value.

13. In the manufacture of quartz oscillator plates the improvement which comprises treating each oscillator plate with radiations from a radio-active substance adapted to decrease its frequency of oscillation, treating each plate to the action of ultra-violet light rays adapted to increase its frequency of oscillation, and terminating the treatment of each plate with said ultra-violet light rays when its frequency of oscillation reaches a predetermined value.

14. In the manufacture of quartz oscillator plates, the improvement which comprises heating each oscillator plate to an elevated temperature to sensitize it to frequency change, treating each sensitized plate to the action of radiations from a radio-active substance adapted to decrease its frequency of oscillation, and terminating the treatment of each plate with said radiations from a radio-active substance when its frequency of oscillation reaches a predetermined value.

15. In the manufacture of quartz oscillator plates, the improvement which comprises heating each oscillator plate to an elevated temperature to sensitize it to frequency change, treating each sensitized plate to the action of radiations from a radio-active substance adapted to decrease its frequency of oscillation, treating each plate to the action of ultra-violet light rays adapted to increase its frequency of oscillation, and terminating the treatment of each plate with said ultra-violet light rays when its frequency of oscillation reaches a predetermined value.

16. In the manufacture of quartz oscillator plates, the improvement which comprises heating each oscillator plate to an elevated temperature to sensitize it to frequency change, treating each sensitized plate to the action of radiations from a radio-active substance adapted to decrease its frequency of oscillation, heating each oscillator plate so treated to increase its frequency of oscillation, and terminating the heating of each plate when its frequency reaches a predetermined value.

17. In the manufacture of oscillator plates the step comprising decreasing the frequency of the oscillator plate by treating the same with radiations from a radio-active substance.

CLIFFORD FRONDEL.